

## UNITED STATES PATENT OFFICE

1,963,493

PROCESS OF REVIVIFYING BRUCITE OR  
MAGNESIUM HYDROXIDEEmerson C. Higgins, Jr., West Los Angeles, Calif.,  
and Franklin T. Gardner, Tulsa, Okla.No Drawing. Application September 16, 1931,  
Serial No. 563,220

10 Claims. (Cl. 23—201)

The present invention relates to a process for the revivification of brucite or magnesium hydroxide that has been employed in the purification of hydrocarbons such, for example, as 5 cracked gasoline or its equivalent.

The process is particularly directed to the treatment of brucite, or other forms of magnesium hydroxide, particularly such as is described in connection with copending patent application 10 of Emerson C. Higgins, Jr. and Franklin T. Gardner, Serial No. 543,004, filed June 8, 1931.

One of the objects of the present invention is to remove, from the used brucite, silica, silicates or silicic acid that form within and on the 15 surface of the particles of the brucite during the reactions which take place when gasoline or other similar hydrocarbon material is passed over the same for the purpose of rendering said hydrocarbons "sweet to doctor".

20 In the said above mentioned copending application there has been described a process which, in essence, consists in treating a hydrocarbon such as gasoline so as to modify the therein contained mercaptans, thereby rendering the treated 25 gasoline or other hydrocarbon "sweet to doctor", so that it may be readily merchantable. In the said process the gasoline or other hydrocarbon is passed, in admixture with sulphur dissolved therein, upwardly through a bed of comminuted 30 brucite or through artificial magnesium hydroxide. In the presence of the sulphur, the mercaptans in the gasoline or other hydrocarbons react with the magnesium hydroxide or brucite to finally form organic disulphides. During the 35 course of this process the brucite gradually loses its efficacy and becomes coated and permeated with silicates, or more particularly with free silicic acid. This silicic acid is derived from the silicates present in the natural brucite and other 40 forms of magnesium hydroxide, which silicates usually consist of those of iron, magnesium, calcium, aluminum, potassium, etc.

45 While the presence of these silicates in the fresh, or unused, brucite does not interfere materially with the operation of the sweetening, as disclosed in the said copending application, the reactions taking place during the said operations do, however, decompose these silicates with the formation of the corresponding sulphides or sulphates of the said metals and the liberation of 50 free silicic acid. The latter is a very gelatinous material and deposits itself upon the surface of the brucite, thereby retarding the efficacy of the latter, so that, as the operation of purifying the 55 gasoline proceeds, the brucite gradually loses its efficacy and thus brings about the requirement for its revivification.

There has been described, in the said copending application, a comparatively simple process 60 of brucite revivification, which consists in the

treatment of the brucite with either hot or cold water and/or steam for the removal of the soluble sulphides or sulphates therefrom. While this treatment with hot water serves for the removal of water-soluble materials, it will not remove the 65 free silicic acid, for the reason that the latter is not readily soluble in water.

The specific object of the present invention, therefore, is the removal of this gelatinous silicic acid that remains upon the brucite. It is known 70 that silicic acid is soluble in concentrated alkaline solutions, but dilute solutions of alkalies may be employed provided that elevated temperatures are employed. It has been found that very excellent results can be obtained by the use of a 75 2.5% solution of caustic soda (sodium hydroxide, NaOH). Approximately the temperature of boiling water is used during the first stage of revivification of the brucite, when performed in accordance with the present invention. It is not 80 necessary to remove the brucite from the towers in which it is stored during the gasoline sweetening process disclosed in the copending application, Serial No. 543,004, as the revivifying treatment can be carried out in said tower itself. It 85 is effected as follows:

After the gasoline or other hydrocarbon has been displaced by a slowly rising column of water so as to drive the hydrocarbon out of the tower ahead of it, the water is then withdrawn and 90 a caustic soda solution, say one containing substantially 2.5% by weight of sodium hydroxide, NaOH, is forced into the bottom of the tower until the entire mass of brucite is submerged. The mixture in the tower is then heated to boiling by means of a closed steam coil, the design and further purpose of which is hereinafter described. The hot or boiling solution of caustic soda in the tower is allowed to act upon and react with the silicic acid on and in the brucite 95 for a period of from 4 to 6 hours, following which the caustic soda solution, now containing a solution of sodium silicate, is drawn out of the tower. Following this, the brucite in the tower is then washed with hot water to remove the 100 soluble sulphates or sulphides which may have escaped solution during the previous treatment. The water which is used after the removal of the sodium silicate solution is allowed to act upon the brucite for 3 to 4 hours and is then drawn 105 off. It is within the scope of the present invention to repeat this washing operation with hot water, or merely to rinse the brucite once or twice so as to insure the removal of as much as possible of the adhering solution.

110 After the wash-water has been drained from the tower, hot or cold air is passed through the mass of brucite to assist in drying the same. Each tower is equipped with a closed coil, through which either live or exhaust steam is passed. 115

120

This coil is designed and located in the tower so as to obtain the most effective drying of the brucite. After the brucite is dried, it is ready for re-use, and fresh quantities of gasoline to be purified may then be passed through the same in the manner disclosed in the already mentioned copending application, Serial No. 543,004, filed June 8, 1931.

Experiments have demonstrated that after the 10 revivification of a given mass of brucite has been effected three or four times with the use of the caustic sodium solution, there will be practically no more silicates present in the brucite, and the brucite may then subsequently be revivified for use merely by the expedient of washing 15 it with hot water and subsequent drying as set forth in the said copending application. It has also been found that such desilicized brucite is much more efficient than the natural 20 brucite, and it is within the scope and intent of the present invention to subject natural brucite to a treatment with caustic soda in the manner above described for the purpose of rendering the same more active than it would otherwise be for effecting the sweetening and neutralization 25 of hydrocarbons.

However, it is more economical to depend upon the reaction between the impurities in the gasoline or hydrocarbon and the silicates in the 30 natural brucite, rather than to expend time and reagents to remove these before initially using the brucite. If this is desired, however, brucite may be treated with a strong acid to convert the 35 therein contained silicates into free silicic acid, following by washing to remove the salts formed thereby, and then to remove the thus liberated silicic acid by means of a solution of a caustic soda in the manner already hereinabove set forth.

40 While a solution of caustic soda is the most economical and generally available for effecting the removal of the gelatinous silicic acid from the brucite, it will, of course, be obvious to a skilled chemist that a similar reaction will take place if said gelatinous silicic acid be subjected to the action of one of the other elements of the alkali groups of which lithium is the first member, the others being sodium, potassium, caesium and rubidium. It is therefore within the 45 intent and scope of the present invention to employ such other alkalies and particularly potassium hydroxide, which in some parts of the world is available at a cost not very much higher than that of sodium hydroxide. For practical purposes, however, the other alkalies in this group, 50 while capable of performing the function of removing the silicic acid from the brucite, are too expensive at the present time for commercial exploitation.

60 While the operations are most economically carried out in the tower in which the brucite has been used for effecting the sweetening of gasoline or other hydrocarbons, it will, of course, be within the scope of the present invention to perform said operations outside of said tower after removing the brucite from the tower into any suitable container that is not adversely affected by the caustic soda solution employed in the revivifying treatment.

70 What it is desired to protect by Letters Patent is the following:

1. The process of treating brucite which comprises subjecting the same to the action of a di-

lute alkaline solution of the type of sodium hydroxide solution while under superatmospheric temperature to effect the removal of silicious matter therefrom.

2. The process of treating brucite which comprises subjecting the same to the action of a boiling solution of the hydroxide of a metal of the alkali group to remove silicious matter therefrom. 80

3. The process of treating brucite which comprises subjecting the same to the action of a boiling solution of sodium hydroxide to remove silicious matter therefrom. 85

4. The process of revivifying spent brucite which has been employed in the purification of hydrocarbons which comprises boiling the same with an alkaline solution, then withdrawing said solution, then boiling the brucite with water, withdrawing the water, and drying the brucite. 90

5. The process of revivifying spent magnesium hydroxide employed in the sweetening of hydrocarbons by which sweetening the magnesium hydroxide becomes inactivated by deposition of salts and silicic acid thereon, which comprises converting said silicic acid into a soluble compound thereof, and dissolving said compound by 100 means of water, withdrawing the resulting solution and drying the magnesium hydroxide. 95

6. The process of revivifying spent magnesium hydroxide which has become inactive by contact with impure hydrocarbons due to the deposition of silicic acid thereon, which comprises the step of subjecting said magnesium hydroxide to the action of a caustic alkali. 105

7. The process of revivifying spent magnesium hydroxide which has been employed in the purification of hydrocarbons which comprises: treating the spent magnesium hydroxide contaminated with silicic acid with a dilute alkaline solution whereby contained silicic acid is converted into a water soluble silicate, then separating the silicate from the hydroxide by washing with water. 110

8. The process of enhancing the purifying power of brucite for hydrocarbons which comprises converting the silicates naturally contained in the brucite into metallic salts and free silicic acid by heating the brucite with a strong acid capable of causing such conversion without affecting the brucite, converting the silicic acid into a water soluble silicate by the contact therewith of a hydroxide of a metal of the alkali group, then washing the thus formed silicate out from the brucite with water. 115

9. The process of enhancing the purifying power of brucite for hydrocarbons which comprises converting the silicates naturally contained in the brucite into metallic salts and free silicic acid by heating the brucite with a strong acid capable of causing such conversion without affecting the brucite, converting the silicic acid into a water soluble sodium silicate by the contact therewith of sodium hydroxide, then washing the thus formed silicate out from the brucite with water. 120

10. The process of revivifying spent magnesium hydroxide which has become inactive by contact with impure hydrocarbons due to the deposition of silicic acid thereon which comprises the step of subjecting said magnesium hydroxide to the action of a solution of sodium hydroxide of about 2:5% concentration. 125

135

EMERSON C. HIGGINS, JR.  
FRANKLIN T. GARDNER.